

S. J. Potter.

Railroad Rail Pile.

No 60,783.

Patented Jan. 1, 1867.

Fig. 2.



Fig. 1.



Fig. 3.



Witnesses.

Geo. W. Rootwell  
Colonel C. Remond.

Exxonitor:

S. L. Potter  
By O'Kright & Co.  
Albion & Co. Atty.

# United States Patent Office.

SAMUEL L. POTTER, OF WYANDOTTE, MICHIGAN.

*Letters Patent No. 60,783, dated January 1, 1867.*

## IMPROVEMENT IN FAGGOTS FOR RAILROAD RAILS.

The Schedule referred to in these Letters Patent and making part of the same.

TO ALL WHOM IT MAY CONCERN:

Be it known that I, SAMUEL L. POTTER, of Wyandotte, in the county of Wayne, and State of Michigan, have invented a new and improved Rail-Pile; and I do hereby declare that the following is a full, clear, and exact description thereof, which will enable those skilled in the art to make and use the same, reference being had to the accompanying drawings, forming part of this specification, in which—

Figure 1 represents a transverse section of my improved pile or faggot, one-half the actual size.

Figure 2 is a transverse section of the same, illustrating a manner of applying old railroad bars in place of the inner or intermediate iron bars of the pile.

Figure 3 represents a transverse section of the complete rail, full size.

Similar letters of reference indicate corresponding parts.

This invention consists in forming a pile, from which railroad rails are drawn or rolled, of bars of iron and steel, arranged or disposed substantially as hereinafter described, and in such a manner that the rail will be rolled with a steel head, the latter protected from undue heating, and the iron and steel perfectly welded together by the rolling operation.

In fig. 1 *a a* represent two bars of iron, seven inches broad and one and a quarter inch in thickness, and *b* represents four bars of iron, three and a half inches in breadth and one and a quarter inch in thickness. These bars, *a* and *b*, are placed edgewise, side by side, the narrow bars, *b*, leaving a recess to receive a bar, *c*, of steel, five inches in width and three and a half inches in thickness. This steel may be manufactured by the Bessemer or pneumatic process. This pile, thus formed, is rolled edgewise, and a rail produced, as shown in fig. 3, *A* being the steel head, and *B* the iron neck and base. In fig. 2 is shown a pile of the same construction and arrangement, the interior or intermediate iron bars, *b'*, consisting of old railroad rails. By these means it will be seen that the steel will be brought to a welding heat, and fully protected by the iron, as the steel will weld at a much lower heat than the iron, and the two metals will, during the process of rolling, be perfectly welded together.

Having thus described my invention, what I claim as new therein, and desire to secure by Letters Patent, is—

A pile or faggot for rolling railroad bars, constituted of iron and steel bars, arranged substantially as herein represented and described.

SAMUEL L. POTTER.

Witnesses:

JOHN BENNETT,  
WM. H. GRAHAM.